

W. HOSKINS,

METHOD OF RECOVERING TIN.  
APPLICATION FILED APR. 10, 1913.

1,088,422.

Patented Feb. 24, 1914.



## Witnesses:

W. Taylor.  
Chas. H. Buell,

Inventor.

10 William Haskins,  
By appointment of the State of Maine,  
At Boston, Mass.

# UNITED STATES PATENT OFFICE.

WILLIAM HOSKINS, OF CHICAGO, ILLINOIS.

## METHOD OF RECOVERING TIN.

1,088,422.

Specification of Letters Patent. Patented Feb. 24, 1914.

Application filed April 10, 1913. Serial No. 760,124.

To all whom it may concern:

Be it known that I, WILLIAM HOSKINS, a citizen of the United States, residing at Chicago, in the county of Cook and State of Illinois, have invented a new and useful Improvement in Methods of Recovering Tin, of which the following is a specification.

My invention relates to an improved method of producing commercial tin from 10 more or less oxidized tin or tin alloys.

In the process of winning tin from tin-plate scrap, for example, a product is obtained consisting of a mixture of finely divided tin and tin oxid, which has always 15 been difficult heretofore to convert into commercial tin; and one of my objects is to provide a simple and improved method of economically treating said product. My improved method may also be employed to advantage in the production of commercial tin from drosses produced in the manufacture of tin-plate, and from type-metal, both of which contain tin or tin alloy and oxid thereof.

For the practice of my improved method I provide a furnace having an upright chamber equipped with twyters at different levels, the twyters having valves whereby the air supply at each of said levels may be regulated. I charge the furnace with carbon to a level above the upper twyters and by means of the valves the volume of air forced in at each of the twyter levels is so regulated as to maintain the mass of carbon incandescent 35 throughout, but at temperatures increasing with the height of the level. The metal oxid or mixture of the metal and its oxid is fed into the top of the furnace and subjected to the action of the upper hottest zone 40 in a reducing atmosphere which quickly reduces the highly refractory oxid of tin to metal and melts the metal causing it to run down through the lower zones. The said lower zones also contain a reducing atmos- 45 phere, but of diminishing temperatures which serve to maintain the metal in molten condition without danger of reoxidation. The molten metal is allowed to escape through an opening in the lower end of the 50 furnace wall where it is collected in a suitable basin or "float."

In the accompanying drawing which illustrates a furnace suitable for carrying out

my improved method Figure 1 is a vertical section of the furnace taken on line 1 in Fig. 55 2; and Fig. 2 is a plan section taken on line 2 in Fig. 1.

The vertical walls 3 of the furnace are of fire-brick inclosing an upright chamber 4. At the lower end of the chamber is an iron 60 base-plate 5 having a slight inclination, and above the lower end thereof is an outlet opening 6 in the furnace wall. Below the opening 6 is a basin or float 7. The furnace illustrated is equipped with three sets of 65 twyters of which the twyters 8 form the upper set, the twyters 9 an intermediate set and the twyters 10 the lower set. They extend into the chamber 4 from three sides as indicated and each of the twyters is provided 70 with a hand-operated valve 11 for regulating the supply of air therethrough. The twyters communicate with a bustle pipe 12 which receives air under pressure from a compressor or a compressed air supplier, 75 not shown. Surmounting the chamber 4 is a hook and stack 12 for the escape of gases, leaving an opening 13 below the hood through which the chamber may be charged.

In practice the chamber is filled to approximately the level indicated by the dotted line 14 with charcoal which is ignited and maintained incandescent by the air forced in at the twyters. The valves 11 of the lower twyters 10 are opened only far 80 enough to permit a comparatively small quantity of air to pass therethrough to support combustion of the charcoal in the lower zone adjacent to the twyters 10 causing the generation of carbon monoxide gas which 85 rises upward through the chamber. The valves 11 of the twyters 9 are opened somewhat wider to increase combustion in the zone adjacent to the twyters 9 over that in the lower zone; and the valves 11 of the 90 twyters 8 are opened still wider to effect still more rapid combustion of the carbon in the zone adjacent to the twyters 8. Thus the temperature is greatest in the upper part of the furnace chamber and diminishes 95 toward the lower end thereof, while a reducing atmosphere is maintained throughout the chamber. The tin or tin alloy and oxides thereof are shoveled into the chamber 4 through the opening 13 and are subjected in 100 105 the upper zone to a melting temperature in

a reducing atmosphere which effects quick deoxidation of the metal oxids and melts the metal. The latter as it is melted percolates downward through the incandescent mass in the zones 9 and 10 which maintains the metal in a molten state and against re-oxidation. As the molten metal descends to the base plate 5 it flows out through the opening 6 into the "float" 7. Any unconsumed charcoal and unreduced oxids escaping from the chamber into the float may be skimmed off and returned to the furnace. As metallic impurities in the tin as a rule are heavier than tin, they descend to the bottom of the float 7, leaving the tin in a commercially pure condition overlying the impurities. It becomes an easy matter therefore to ladle the tin out of the float into molds to form ingots of commercially pure tin.

The valves 11 make it possible to suitably control the temperatures at the different zones. The upper zone should in practice be maintained at a temperature which, while exceeding the melting point of tin, will not effect volatilization thereof and consequent loss by escape through the stack. The heat of the lower zone should be below that of the upper zone and so controlled that the molten tin will run out into the "float" at a temperature neither too high nor too low, otherwise it is apt to be brittle and have its color and luster impaired. By manipulating the valves 11 the operator may so regulate the temperature as to obtain the best results and maintain an output of uniformly high grade.

What I claim as new and desire to secure by Letters Patent is—

1. The herein described method of treating a mixture of tin, or tin alloys, and their oxids, which consists in subjecting the same in a reducing atmosphere to a temperature exceeding the fusing point of tin, to reduce the oxids and melt the metal, then passing the molten metal through a reducing atmosphere of a temperature lower than that first named.

2. The herein described method of treating a mixture of tin, or tin alloys, and their oxids, which consists in subjecting the same in a reducing atmosphere to a temperature exceeding the fusing point of tin, to reduce the oxids and melt the metal, then passing the molten metal downward through zones of reducing atmosphere of progressively decreasing temperatures.

3. The herein described method of treating a mixture of tin, or tin alloys, and their oxids, which consists in maintaining incandescent a bed of carbon by introducing air into the same at different levels and in progressively decreasing quantities in the downward direction, introducing the mixture to be treated upon the top of the bed, reducing the oxids and melting the metal and causing it to percolate through the progressively decreasing heat zones in the bed, and discharging the molten product from the base of the bed.

WILLIAM HOSKINS.

In presence of—

DAISY C. THORSEN,  
OTTILIE C. AVISUS.